

No. 797,505.

PATENTED AUG. 15, 1905.

I. EISENSTEIN.

METHOD OF FINISHING CANES AND THE LIKE AND ARTICLE PRODUCED  
THEREBY.

APPLICATION FILED MAR. 11, 1905.



Witnesses

J. M. Fowler Jr.  
Edwin E. Vrooman.

Inventor

Israel Eisenstein,  
By  
Mason, Hammick & Sawyer,  
his Attorneys.

# UNITED STATES PATENT OFFICE.

ISRAEL EISENSTEIN, OF NEW YORK, N. Y.

## METHOD OF FINISHING CANES AND THE LIKE AND ARTICLES PRODUCED THEREBY.

No. 797,505.

Specification of Letters Patent.

Patented Aug. 15, 1905.

Application filed March 11, 1905. Serial No. 249,626.

*To all whom it may concern:*

Be it known that I, ISRAEL EISENSTEIN, a citizen of the United States, residing at New York, in the borough of Manhattan and State of New York, have invented certain new and useful Improvements in Methods of Finishing Canes and the Like and Articles Produced Theréby; and I do hereby declare the following to be a full, clear, and exact description of the invention, such as will enable others skilled in the art to which it appertains to make and use the same.

This invention relates to the method of finishing bamboo, tonquin, and reed sticks.

The objects of the invention are to produce bamboo, tonquin, or reed canes with an enameled surface produced by baking the paint, varnish, or other coating on the body of the cane, whereby the enameled surface is produced which is practically impossible to scratch or remove. Heretofore attempts have been made to finish bamboo, reed, and tonquin canes with a suitable paint or varnish; but all such attempts, so far as I am aware, have proved impractical or unsuccessful, owing to the difficulty of securing a firm contact of the coating material onto the glazed or natural covering of such classes of sticks. It is a common practice to sandpaper and polish hard wood and other sticks possessing a porous and a natural unglazed surface; but this class of wood is totally different from sticks or reeds having a natural glazed or sheal covering, such as is found on bamboo, reed, and tonquin sticks. It has been found impractical to bake varnish or paint on porous naturally-unglazed sticks, owing to the fact that the sticks are injured and practically destroyed by such baking. Owing to the natural consistency of bamboo, tonquin, and reed sticks the same are not injured by the baking, and by the use of a specially-prepared varnish or coating which I have devised I am enabled to finish such classes of canes with a hard enameled surface—a result which, as far as I am aware, has never been heretofore successfully accomplished.

In carrying out the method employed in producing the finished surface on canes of such variety I make use of the mechanism illustrated in the accompanying drawings, in which—

Figure 1 is a perspective view of the receptacle for containing the composition used for coating the canes and the draining-receptacle employed. Fig. 2 is a perspective view, shown

partly in section, of a cane-carrying member which is adapted to be positioned within the receptacle depicted in Fig. 1 for covering the canes with the composition employed for coating the same. Fig. 3 is a perspective view of a member constituting a weight. Fig. 4 is an elevated front view of the furnace in which the unfinished canes which are coated with the composition contained in the receptacle depicted in Fig. 1 are to be baked for enameling the same. Fig. 5 is a longitudinal sectional view of a finished cane constructed in accordance with the present invention.

The varnish paint preferably employed in the present invention comprises caoutchouc, six parts; rectified spirits of turpentine, twelve and one-half parts, and rectified shale-naphtha, fifteen parts. The mentioned three ingredients are then stirred and heated on a sand bath. I then take of the above mixture seventy-five per cent. and mix therewith pale boiled oil seventy-five per cent. and pale copal varnish one hundred per cent. This mixture of all of the ingredients is then heated to 190° from ten to twelve hours. The coloring-matter for the varnish is mixed before heating.

After the varnish has been made the desired amount is deposited in the receptacle 1. The body 2 of the canes, which is formed of bamboo, tonquin, or reed sticks, is then placed within the cane-carrying member 3. Said member 3 comprises a frame which is provided with parallel members 4, secured to the lower portion thereof. The members 4 constitute the bottom of the member 3. Each member 4 is provided with upwardly-projecting pins 5. Each of said pins 5 is engaged by the lower end of the body of an unfinished cane. The upper end of the member 3 is closed by netting 6, preferably formed of metallic material. Within each mesh of the cover 6 one of the unfinished canes is positioned. It is desirable that the covering 6 be provided with the same number of meshes as there are pins secured to the transverse members 4 in the lower portion of the frame of the cane-carrying member 3. An unfinished cane is secured within one of the meshes of the covering 6 and upon one of the pins 5 of a member 4. When the cane-carrying member 3 is positioned within the receptacle 1, it has been found that the canes will float if they are not weighted down, and to obviate this removal of the canes from within the carrying member I employ a weighted member 7, preferably formed of metal, which is positioned upon the

handles of the cane-bodies for pressing them down and retaining the same within the mesh or apertured covering and upon the pins of members 4. The cane-carrying member is suspended upon any suitable traveling means—as, for instance, a traveling pulley—by means of cable 8, which is connected to the sides of the frame constituting member 3 by means of extending members 9, which are preferably secured near the corners of the upper portion of the frame. It will be necessary after the canes are positioned within the member 3 to lift the same and move it over the receptacle 1 and subsequently lower the same into said receptacle for immersing the bodies of the canes in the varnish contained within said receptacle. After the canes have been covered by the varnish the cane-carrying member 3 is then lifted and positioned over the draining-receptacle 10 and lowered upon the frame 11 supported thereby. The frame 11 is positioned above the receptacle 10. Frame 11 comprises parallel sides and ends and a transverse connecting member 12. The cane-carrying member 3 is rested upon the frame 11, carried by the draining-receptacle 10, for permitting of the cane-bodies to be drained before the cane-carrying member containing the cane-bodies is placed in the oven of the furnace 13 for baking the varnish upon the cane-bodies for producing an enameled coating thereon. It will be obvious that the cane-bodies after they have been varnished may be removed from the cane-carrying member 3 and separately placed in the oven for baking the varnish placed thereon. The cane-bodies may be supported in the oven at each of their ends or may be suspended by means of their handle structure upon any suitable support. In the event of gases accumulating in the furnace I have provided a valve 14, which is actuated by a flexible member 15, for permitting of the escape of said gases.

The glazed or substantially non-porous surface of the bamboo, tonquin, or reed sticks is entirely covered by the enameled coating 15, formed by baking the varnish in the oven of the furnace 13. The body of the cane after it has been coated with my improved varnish is placed in the oven as specified and the temperature in said oven maintained from about 200° to 300° of heat for not less than three hours.

I have found by numerous tests that it is practically impossible to secure a finish on a glazed reed, bamboo, or tonquin stick unless

the heat is raised to a temperature of not less than 200° and not over 300° for a period of not less than three hours. If the canes are subjected to a heat of more than 300°, the same will be so injured as to be useless for practical purposes, and if subjected to heat for less than three hours the varnish paint will not be properly baked onto the glazed surface. It is impractical to bake ordinary wooden sticks which are not provided with a natural glazed surface, for the reason that said sticks cannot withstand the heat to which they are subjected during the process of baking the varnish paint thereon. My invention does not relate to the finishing of this class of sticks. The object which I had in mind and which I have successfully accomplished and which I have never known to have been successfully accomplished by any other was to provide a method by which the finish could not be scratched after the baking operation is completed. The result I have obtained was accomplished after many experiments both as to the degrees of heat and the length of time the heating should be continued.

I do not wish to limit my invention to any particular mechanical means for carrying out the method or to the particular ingredients employed in the varnish-paint composition, though those which I have set forth I have found to be practical for carrying out the method, as the present invention has reference entirely to the method of finishing bamboo, tonquin, and reed sticks.

What I claim is—

1. The herein-described method of finishing bamboo, tonquin and reed sticks which consists in coating the same in their natural state with a suitable baking varnish paint and subjecting the coated sticks to a temperature of from 200° to 300° of heat for not less than three hours.

2. The herein-described method of finishing bamboo, tonquin and reed sticks which consists in coating the same in their natural state with a suitable baking varnish paint and subjecting the coated sticks to a temperature of from 240° to 300° of heat for not less than three hours.

In testimony whereof I affix my signature in presence of two witnesses.

ISRAEL EISENSTEIN.

Witnesses:

MORRIS OAKLANDER,  
MORRIS BERG.